

## UNITED STATES PATENT OFFICE

1,940,265

## AGENT AND PROCESS FOR DRENCHING SKINS

Wilhelm Neugebauer, Wiesbaden-Biebrich, Germany, assignor to Kalle & Co. Aktiengesellschaft, Wiesbaden-Biebrich, Germany

No Drawing. Application January 15, 1932,  
Serial No. 586,968, and in Germany January 24,  
1931

3 Claims. (Cl. 149—3)

The present invention relates to agents and a process for drenching skins.

Drenching agents containing proteolytic enzymes, for instance those of the pancreas, are already known. The known drenching agents of this kind consist of mixtures of proteinases and amino- and carboxypeptidases, which constituents it was hitherto hardly possible to separate from one another.

10 The present invention is based on the discovery that solutions of pancreas proteinases free from peptidases, and particularly from carboxypeptidases, constitute drenching agents giving a particularly good drenching effect. The 15 skins drenched with these proteinases and the leathers produced therefrom have, as compared with those drenched with a mixture of proteinases and peptidases, a more compact and softer touch without, however, being flabby.

20 The proteinases free from peptidases can be utilized in the same manner as the drenching agents hitherto used. For the neutralization of the alkalinity of the skins coming from the lime liquor, the usual buffering agents may be 25 employed, such as ammonium salts, for instance ammonium sulfate or ammonium chloride, or lactic acid, boric acid, sodium bisulfite or other substances having a similar action. The said agents may be employed in a preliminary bath 30 before the drenching process or alternatively,—particularly in the case of ammonium salts—they may be applied in the drenching solution itself.

The proteinases free from peptidases, which 35 are utilized in the present process; can for instance be obtained according to the process set forth in the British Patent Specification No. 356,638, dated January 31, 1930, in the name of Kalle & Co. Aktiengesellschaft.

40 The following examples illustrate the invention:

1. 0.1 kilo of ammonium chloride and a quantity of proteinase free from peptidase obtained from hog's pancreas by the process according to the specification above-mentioned,

are dissolved in 60 liters of water. The quantity of enzyme employed is such that 1.0 kilo of gelatine after treatment therewith for 1 hour at 37° C., no longer solidify on cooling. 20 kilos of limed, unhaired and rinsed calf skins 60 of normal quality are treated with this solution for 1 hour at about 37° C.

By that time the pelts will have become drenched. After being worked up in the usual manner, they yield a leather of a softer and 65 more compact touch than a leather which has been drenched with the natural mixture of proteinases and peptidases of hog's pancreas.

2. 20 kilos of unhaired goat skins are treated for ½ hour at about 38° C. in a reel with 100 70 liters of water and 0.2 kilo of a mixture of ammonium sulfate and pancreas proteinase free from peptidase. The quantity of enzymes contained in the mixture is such as to be capable of liquefying 2.5 kilos of gelatine at 37° C. after 75 an hour's action. After having been drenched, the skins are worked up in the usual manner. An excellent leather is thus obtained.

3. 20 kilos of limed and unhaired calf pelts are stirred in a bath consisting of lactic acid 80 of ½ to 1% strength until a test portion cut from the pelt only yields a slight red coloration with phenolphthaleine. The skins are then taken out of the bath, rinsed and treated with a drenching agent as indicated in Example 1. 85 The quantity of ammonium chloride usually added may be reduced or even omitted.

I claim:

1. The process of drenching skins which consists in causing a solution of pancreas proteinases free from peptidases to act upon the skins. 90
2. The process of drenching skins which consists in causing a solution of pancreas proteinases free from peptidases containing an addition of buffering agents to act upon the skins. 95
3. As a new drenching agent, a solution of pancreas proteinases free from peptidases. 100

WILHELM NEUGEBAUER. 100